# EUROPEAN PATENT SPECIFICATION

(11) **EP 4 332 998 B1**
(45) Date of publication and mention of the grant of the patent: **25.02.2026**
(21) Application number: 23193064.5
(22) Date of filing: 23.08.2023
(51) Int. Cl.: H01F 1/057, H01F 41/02

(54) **CE-CONTAINING SINTERED NDFEB MAGNET AND MANUFACTURING METHOD THEREOF**
CE-HALTIGER GESINTERTER NDFEB-MAGNET UND HERSTELLUNGSVERFAHREN DAFÜR
AIMANT NDFEB FRITTÉ CONTENANT DU CE ET SON PROCÉDÉ DE FABRICATION

(30) Priority: 30.08.2022 CN 202211047034
(43) Date of publication of application: 06.03.2024
(73) Proprietor: Yantai Dongxing Magnetic Materials Inc., Yantai City 265500 (CN)
(72) Inventor: Chen, Xiulei, Yantai City, 265500 (CN); Peng, Zhongjie, Yantai City, 265500 (CN); Dong, Zhanji, Yantai City, 265500 (CN); Ding, Kaihong, Yantai City, 265500 (CN); Xu, Xiandong, Yantai City, 265500 (CN)
(74) Representative: Gulde & Partner

(56) References cited:
- WO-A1-2020/233316
- CN-A- 104 575 920
- CN-B- 111 210 963
- ZHANG YUJING ET AL: "Effects of REFe2on microstructure and magnetic properties of Nd-Ce-Fe-B sintered magnets", ACTA MATERIALIA, ELSEVIER, OXFORD, GB, vol. 128, 1 February 2017 (2017-02-01), pages 22 - 30, XP029944496, ISSN: 1359-6454, DOI: 10.1016/J.ACTAMAT.2017.02.002

## Description

### BACKGROUND OF THE INVENTION

### Field of the Invention

The present invention relates to a Ce-containing and sintered NdFeB magnet and a corresponding manufacturing method thereof.

### Description of the Prior Art

Elements with high abundance, such as La and Ce, are often doped into NdFeB magnets for price reasons. However, since La and Ce have lower magnetic performance parameters, this leads to a significant decrease in magnetic performance after addition. To optimize such magnets, the industry has adopted a multi-principal phase process, surface grain boundary diffusion and other ways to optimize magnets.

CN102800454A relates to a low-cost dual-phase Ce permanent magnet alloy and a preparing method thereof, which can obtain higher magnetic properties by forming Nd-Fe-B and (Ce, Re)-Fe-B phases. However, the magnetocrystalline anisotropy field constant (HA) of the (Ce, Re)-Fe-B principal phase in this method is reduced too much, which limits the improvement of magnetic properties.

WO 2020/233316 A1 relates to a method of diffusing rare earth elements into the basic magnet which contains a CeFe₂ phase. Thereby, the magnetic performance of the CeFe₂ phase can be enhanced by transforming the same into an REFe₂ phase. However, REFe₂ easily appears in the grain boundary phase with high proportion addition of Ce. Further, the single REFe₂ phase has weak magnetic isolation effect, which reduces the coercivity of magnet.

Y. Zhang et al., Acta Mater. 2017, 128, 22-30 relates to the effects of REFe₂ on microstructure and magnetic properties of Nd-Ce-Fe-B sintered magnets. The publication states that by sintering of the green compacts above the melting point of the REFe₂ phase, densification of the magnet and the formation of continuous and smooth grain boundary phases is promoted.

### SUMMARY OF THE INVENTION

The invention is defined by the appended claims. The description that follows is subjected to this limitation. Any disclosure lying outside the scope of said claims is only intended for illustrative as well as comparative purposes.

In particular, the present invention relates to a Ce-containing and sintered NdFeB magnet as defined in claim 1 and a corresponding manufacturing method thereof as defined in claim 5.

Further aspects of the present disclosure could be learned from the dependent claims or the following description.

### BRIEF DESCRIPTION OF THE DRAWING

Features will become apparent to those of ordinary skill in the art by describing in detail exemplary embodiments with reference to the attached drawings in which:
Figure 1 is a schematic diagram of magnet with a multi-layered grain boundary structure.
Figure 2 is an image obtained by high-angle annular dark-field imaging in scanning transmission electron microscopy (HAADF-STEM) and energy-dispersive X-ray spectroscopy (EDS) of a grain boundary location of the magnet of Implementing Example 1.

### DETAILED DESCRIPTION

Reference will now be made in detail to embodiments, examples of which are illustrated in the accompanying drawings. Effects and features of the exemplary embodiments, and implementation methods thereof will be described with reference to the accompanying drawings. In the drawings, like reference numerals denote like elements, and redundant descriptions are omitted. The present disclosure, however, is limited by the scope of the appended claims.

### General Concept

The present invention provides a Ce-containing and sintered NdFeB magnet comprising grains composed of a RE₂Fe₁₄B-type main phase and a multi-layered grain boundary structure between the grains. The multi-layered grain boundary structure includes or consists of - from outside to inside of the multi-layered grain boundary structure and in direct order - layers composed of (or consisting of) the following phases: a RE-rich phase, a Fe-rich phase, and a REFe₂ phase. RE is a rare earth metal including Ce and at least one of Nd and Pr. A weight content of Ce at the magnet alloy composition (i.e. the sum of all elements forming the alloy of the sintered NdFeB magnet) is in the range of 3.00wt.% to 15.00wt. %.

Thus, the sintered NdFeB magnet is a rare earth iron alloy of RE₂Fe₁₄B-type. The main phase of the alloy has a composition of two rare earth atoms (RE) to 14 iron atoms with one boron atom. Cobalt is partially substituted for iron to improve high temperature performance. Besides at least Nd and/or Pr, the magnet alloy includes Ce as rare earth mandatory elements in an amount of 3.00wt.% to 15.00wt.% based on a total weight of the magnet alloy composition. The magnet alloy may also include other rare earth metals, for example Dy and Tb. Furthermore, the magnet alloy may include other metallic or non-metallic alloy components that can be added to optimize the magnet properties for the particular application. Metallic alloy components include Al, Cu, Ga and Ti, and non-metallic alloy components may include small amounts of, for example, H, C, F, N and O.

The sintered NdFeB magnet has a RE-T-B-M magnet alloy composition where
RE is a rare earth metal including Ce and at least one of Nd and Pr;
T is one or both of Fe and Co;
B stands for boron;
M is one or more element selected from the group consisting of Al, Cu, Ga, and Ti;
and wherein the weight contents of the RE-T-B-M magnet alloy composition are set as follows:
   RE: 28.50wt.% to 35.00wt.%, preferably 29.50wt.% to 34.00wt.%, in particular 30.10wt.% to 33.50wt. %;
   Ce: 3.00wt.% to 15.00wt.%; preferably 5.00wt.% to 10.00wt.%;
   Nd and Pr: 14.00wt.% to 29.00wt.%, preferably 15.00wt.% to 28.00wt.%, in particular 15.30wt. % to 27.10wt. %;
   B: 0.70wt.% to 1.20wt.%, preferably 0.80wt.% to 1.10wt.%, in particular 0.85wt.% to 1.05wt. %;
   Co: 0.10 wt. % to 3.00wt. %, preferably 0.50 wt.% to 2.00wt. %;
   M: 0.10wt.% to 3.00wt.%, preferably 0.30wt.% to 1.50wt.%, in particular 0.55wt.% to 1.20wt.%; and
   the residual is Fe and unavoidable impurities (caused, for example, by condition of manufacturing).

According to a preferred embodiment, the weight contents of Al, Cu, Ga, and Ti as metallic alloy components of the RE-T-B-M magnet alloy composition are independently from each other set as follows:
Al: 0.01wt.% to 1.00wt.%, preferably 0.05wt.% to 0.60wt.%;
Cu: 0.01wt.% to 1.00wt.%, preferably 0.10wt.% to 0.50wt.%;
Ga: 0.01wt.% to 1.00wt.%, preferably 0.10wt.% to 0.50wt.%; and
Ti: 0.01wt.% to 1.00wt.%, preferably 0.10wt.% to 0.40wt.%.

In particular, the Ce-containing and sintered NdFeB magnet may have the following RE-T-B-M magnet alloy composition:
RE: 30.10wt.% to 33.50wt.% and 3.00wt.% to 15wt.% thereof Ce;
B: 0.85wt.% to 1.05wt.%;
Al: 0.05wt. % to 0.60wt. %;
Cu: 0.10wt.% to 0.50wt.%;
Co: 0.50 wt. % to 2.00wt. %;
Ga: 0.10wt. % to 0.50wt.%; and
Ti: 0.10wt. % to 0.40wt.%,
wherein the residual is Fe and unavoidable impurities.

In accordance with the before mentioned embodiments or independently thereof, the compositions of the layers of the multi-layered grain boundary structure are set as follows.

In the RE-rich phase, RE takes an atomic proportion of 50.0at.% to 63.0at.%, preferably 50.2at.% to 62.3at.%, Fe plus Co takes an atomic proportion of 30.0at.% to 40.0at.%, preferably 32.2at.% to 39.7at.%, and M takes an atomic proportion of 2.0at.% to 12.0at.%, preferably 2.2at.% to 10.1at.%, wherein the components plus unavoidable impurities add up to 100at. %.

In the Fe-rich phase, RE takes an atomic proportion of 10.0at.% to 30.0at.%, preferably 12.4at.% to 26.0at.%, Fe plus Co takes an atomic proportion of 65.0at.% to 85.0at.%, preferably 68.1at.% to 81.4at.%, and M takes an atomic proportion of 1.0at.% to 7.0at.%, preferably 1.3at.% to 6.2at.% , wherein the components plus unavoidable impurities add up to 100at.%.

In the REFe₂ phase, RE takes an atomic proportion of 25.0at.% to 35.0at.%, preferably 28.1at.% to 33.8at.%, Fe plus Co takes an atomic proportion of 60.0at.% to 72.0at.%, preferably 61.4at.% to 69.8at.%, and M takes an atomic proportion of 0.5at.% to 6.0at.%, preferably 0.6at.% to 4.8at.% , wherein the components plus unavoidable impurities add up to 100at.%.

In the multi-layered grain boundary structure, the RE-rich phase layer has a thickness of 1nm to 21nm, the Fe-rich phase layer has a thickness of 1nm to 15nm, and the REFe₂ phase layer has a thickness of 8nm to 550nm.

Thus, the magnet includes a multi-layered grain boundary phase structure. A first layer of the multi-layered structure is a RE-rich phase, which is deposited on the main phase grains of the magnet composition. Atomic ratio of rare earth elements is over 50% and atomic ratio of Fe element is less than 50% in the RE-rich phase. This kind of grain phase has poor magnetic conductivity and better magnetic isolation effect during demagnetization. In addition, surface defects of main phase grains are reduced due to the presence of the RE-rich phase with high concentration of rare earth elements. The reverse magnetic domains are difficult to be nucleated.

The second layer of the multi-layered structure is a Fe-rich phase with high concentration of Fe element. But the magnetic conductivity of reverse magnetic domains already gets weaker after passing the first layer of the multi-layered structure.

The third layer of the multi-layered structure is a REFe₂ phase which has weaker magnetic isolation effect compared with the first layer. But the third layer has larger thickness which can also restrain the extension of reverse magnetic domains. The multi-layered grain boundary phase structure improves the magnetic isolation effect and enhanced the coercivity.

### Preparation Method

A manufacturing method of the Ce-containing and sintered NdFeB magnet comprising grains composed of a RE₂Fe₁₄B-type main phase and a multi-layered grain boundary structure between the grains as defined above includes the following steps:
a) Preparing alloy flakes of the magnet alloy composition by a strip casting process, subjecting the alloys flakes to hydrogen decrepitation und pulverizing the product by jet milling to obtain an alloy powder;
b) Pressing the magnetic powder into a green compact under a magnetic field for orientation followed by cold isostatic pressing;
c) sintering the green compact at 950°C to 1100°C for 2 to 15h, preferably at 1000°C to 1050°C for 4 to 12h, for example, 1010°C for a duration time of 6 hours;
d) After sintering, subjecting the obtained sintered NdFeB magnets to a three step annealing treatment, wherein

in a first step of the annealing treatment a temperature is in the range of 600°C to 750°C, preferably 630°C to 730°C, for example 650°C, for 1h to 5h, preferably 2h to 4h, for example 3h,
in a second step of the annealing treatment a temperature is in the range of 800°C to 950°C, preferably 820°C to 930°C, for example 850°C, for 1h to 5h, preferably 2h to 4h, for example 3h, and
in a third step of the annealing treatment a temperature is in the range of 420°C to 560°C, preferably 450°C to 540°C, for example 480°C, for 1h to 5h, preferably 2h to 4h, for example 3h.

A cooling rate in each of the three steps may be at least 10°C/min.

The alloy flakes are separately prepared by the strip casting process using vacuum induction furnace. The alloys of the strip casting are subjected to hydrogen decrepitation and a jet milling process to be pulverized into magnetic powders.

The magnetic powders are then pressed into green compacts under a magnetic field for orientation. The green compacts are subjected to cold isostatic pressing for increasing density and homogeneity.

The temperature interval of the sintering step may be, for example, at 1000°C to 1050°C with a duration time of 4 to 12 hours. In particular, the sintering temperature can be set to 1010°C for a duration time of 6 hours.

After sintering, the magnets are subjected to a three steps of annealing treatment. For example, a first step temperature is between 630°C to 730°C which is near the eutectic point of RE-rich phase. Thereby, the RE-rich phase has a better wettability and is easy to coat around the main phase grains to form a first grain boundary layer.

In a second step of the annealing treatment, the temperature is raised to be between, for example, 820°C to 930°C, which is near the eutectic point of the REFe₂ phase. Rare earth elements can separate out from the REFe₂ phase and diffuse into the RE-rich of the first grain boundary layer, the RE-rich phase then has a higher rare earth element concentration. Thereby, a part of the REFe₂ phase is transformed into a Fe-rich phase because of the reduction of rare earth element concentration. The Fe-rich phase forms the second grain boundary layer.

The residual part of the REFe₂ phase that joins the Fe-rich phase and is farthest from the main phase grains and maintained in its original state. The residual part of the REFe₂ phase forms the third grain boundary layer. The annealing temperature during the third step of the annealing treatment is, for example, in the range of 450°C to 540°C for optimizing the grain boundary distribution.

More preferably, in the Implementing Examples, the first step annealing temperature was set as 650°C and the cooling rate was at least 10°C/min. The second step annealing temperature was set as 850°C and the cooling rate was at least 10°C/min. The third step annealing temperature was set as 480°C and the cooling rate was at least 10°C/min.

### Testing method of the grain boundary phase thickness and composition in the multi-layered structure

The longest continuous grain boundary around the main phase grain was divided into five equal sections by four dividing lines (line 5 in fig.1, left), then the thickness of the separately corresponding grain boundary phases was measured, that means the thickness of the layers consisting of the RE-rich grain boundary phase 2, the Fe-rich grain boundary phase 3, and the ReFe₂ grain boundary phase 4 (cf. Fig 1, right) are determined. Five main phase grains were measured by the method for each sample in total.

Then twenty groups of data were obtained for every sample and averages, minima, and maxima value were summarized.

Further, energy dispersive spectroscopy (EDS) was used to detect the element content in the width center of the dividing lines for different grain boundary phases. Five main phase grains were measured by the same method for the same sample. Twenty groups of data were obtained for every sample and averages of the element contents were summarized.

To have a better understanding of the present invention, the examples set forth below provide illustrations of the present invention. The examples are only used to illustrate the present invention and do not limit the scope of the present invention.

### Examples

Alloy flakes were separately prepared by strip casting process using vacuum induction furnace according to composition of Implementing Examples 1 to 4 and Comparative Examples 1 and 2. The alloys were subjected to hydrogen decrepitation under a hydrogen pressure of 0.2MPa for a duration time of 2 hours. And then the alloys were heated to 550°C for dehydrogenation for a duration time of 6 hours.

The alloy flakes after hydrogen treatment were then pulverized to magnetic powders with average particle size of 4.0µm by jet milling. Then the magnetic powders were pressed into green compacts under a 2.0T magnetic field for orientation. The green compacts were subjected to cold isostatic pressing under a pressure of 200MPa. The green compacts were sintered at 1010°C for a duration time of 6 hours in a vacuum furnace.

After cooling to room temperature, the sintered magnets were reheated to 650°C for a duration time of 3 hours and then cooled to room temperature with a cooling rate at least 10°C/min. Then the magnets were reheated to 850°C for a duration time of 3 hours, after which the magnets were cooled to room temperature with a cooling rate at least 10°C/min. At last the magnets were reheated to 480°C for a duration time of 3 hours and then cooled to room temperature with a cooling rate at least 10°C/min.

The annealed magnets were machined into cylinders for magnetic testing. Transmission electron microscope (TEM) and energy dispersive spectroscopy (EDS) were used for analysing the microstructure.

Composition and magnetic performance information of the samples is summarized in Table 1, thickness of various grain boundary phases in the multi-layered structure are summarized in Table 2, element contents of RE-rich phase are summarized in Table 3, element contents of Fe-rich phase are summarized in Table 4, element contents of REFe₂ phase are summarized in Table 5.

**Table 1 - Composition and magnetic performance of the magnets**

| | element composition (wt.%) | | | | | | | | | | magnetic properties | |
|---|---|---|---|---|---|---|---|---|---|---|---|---|
| | Al | B | Co | Cu | Fe | Ga | Nd/Pr | Ti | Ce | ΣRe | Br(T) | Hcj (kA/m) |
| Implementing Example 1 | 0.05 | 0.92 | 0.90 | 0.15 | bal. | 0.20 | 24.30 | 0.15 | 6.00 | 30.30 | 1.38 | 995.80 |
| Implementing Example 2 | 0.60 | 1.05 | 0.50 | 0.10 | bal. | 0.10 | 27.10 | 0.40 | 3.00 | 30.10 | 1.39 | 1313.40 |
| Implementing Example 3 | 0.10 | 0.85 | 2.00 | 0.50 | bal. | 0.50 | 26.50 | 0.10 | 7.00 | 33.50 | 1.29 | 1277.58 |
| Implementing Example 4 | 0.05 | 0.92 | 0.9 | 0.15 | bal. | 0.20 | 15.30 | 0.15 | 15.00 | 30.30 | 1.31 | 827.84 |
| Comparative Example 1 | 0.05 | 0.92 | 0.90 | 0.15 | bal. | 0.20 | 28.30 | 0.15 | 2.00 | 30.30 | 1.41 | 1086.54 |
| Comparative Example 2 | 0.05 | 0.92 | 0.90 | 0.15 | bal. | 0.20 | 12.30 | 0.15 | 18.00 | 30.30 | 1.27 | 644.76 |

**Table 2 - Thickness of grain boundary phase in the multi-layered structure**

| | thickness of RE-rich phase | | | thickness of Fe-rich phase | | | thickness of REFe₂ phase | | |
|---|---|---|---|---|---|---|---|---|---|
| | Max. (nm) | Min. (nm) | Ave. (nm) | Max. (nm) | Min. (nm) | Ave (nm) | Max. (nm) | Min. (nm) | Ave. (nm) |
| Implementing Example 1 | 8 | 1 | 4 | 7 | 2 | 3 | 471 | 9 | 47 |
| Implementing Example 2 | 7 | 1 | 3 | 6 | 1 | 3 | 436 | 8 | 41 |
| Implementing Example 3 | 21 | 2 | 8 | 15 | 2 | 7 | 550 | 12 | 58 |
| Implementing Example 4 | 19 | 1 | 7 | 9 | 2 | 6 | 535 | 11 | 53 |
| Comparative Example 1 | no multi-layered structure | | | | | | | | |
| Comparative Example 2 | no multi-layered structure | | | | | | | | |

**Table 3 - Element composition of RE-rich phase in the multi-layered structure**

| element composition of RE-rich phase (at.%) | | | | | | | |
|---|---|---|---|---|---|---|---|
| | RE (at.%) | Fe+Co (at. %) | Al (at.%) | Cu (at.%) | Ga (at.%) | Ti (at. %) | M(Al+Cu+Ga+Ti) (at.%) |
| Implementing Example 1 | 54.9 | 42.9 | 0.4 | 0.8 | 0.5 | 0.5 | 2.2 |
| Implementing Example 2 | 50.2 | 39.7 | 3.8 | 1.7 | 1.5 | 3.1 | 10.1 |
| Implementing Example 3 | 62.3 | 32.2 | 1.8 | 0.8 | 1.4 | 1.5 | 5.5 |
| Implementing Example 4 | 56.3 | 41.4 | 0.3 | 0.7 | 0.6 | 0.7 | 2.3 |
| Comparative Example 1 | no multi-layered structure | | | | | | |
| Comparative Example 2 | no multi-layered structure | | | | | | |

**Table 4 - Element composition of Fe-rich phase in the multi-layered structure**

| element composition of Fe-rich phase (at.%) | | | | | | | |
|---|---|---|---|---|---|---|---|
| | RE (at.%) | Fe+Co (at. %) | Al (at.%) | Cu (at.%) | Ga (at.%) | Ti (at. %) | M(Al+Cu+Ga+Ti) (at.%) |
| Implementing Example 1 | 19.2 | 79.5 | 0.3 | 0.3 | 0.3 | 0.4 | 1.3 |
| Implementing Example 2 | 12.4 | 81.4 | 3.3 | 0.8 | 0.9 | 1.2 | 6.2 |
| Implementing Example 3 | 26.0 | 68.1 | 1.2 | 2.1 | 1.4 | 1.2 | 5.9 |
| Implementing Example 4 | 22.3 | 75.4 | 0.6 | 0.7 | 0.5 | 0.5 | 2.3 |
| Comparative Example 1 | no multi-layered structure | | | | | | |
| Comparative Example 2 | no multi-layered structure | | | | | | |

**Table 5 - Element composition of REFe₂ phase in the multi-layered structure**

| element composition of REFe₂ phase (at.%) | | | | | | | |
|---|---|---|---|---|---|---|---|
| | RE (at.%) | Fe+Co (at. %) | Al (at.%) | Cu (at.%) | Ga (at.%) | Ti (at. %) | M(Al+Cu+Ga+Ti) (at.%) |
| Implementing Example 1 | 30.1 | 69.3 | 0.2 | 0.2 | 0.1 | 0.1 | 0.6 |
| Implementing Example 2 | 28.1 | 69.8 | 1.1 | 0.2 | 0.4 | 0.4 | 2.1 |
| Implementing Example 3 | 33.8 | 61.4 | 0.8 | 1.7 | 1.4 | 0.9 | 4.8 |
| Implementing Example 4 | 28.5 | 68.1 | 0.6 | 0.8 | 1.0 | 1.0 | 3.4 |
| Comparative Example 1 | no multi-layered structure | | | | | | |
| Comparative Example 2 | no multi-layered structure | | | | | | |

The Ce additive weight ratio of Implementing Example 1 was 6.0%, and the sample had a Br of 1.38 T, and a Hcj of 995.80 kA/m.

The Ce additive weight ratio of Implementing Example 4 was as high as 15.0wt%. Hcj was still 827.84 kA/m.

In the magnet of Implementing Examples 1 to 4 there exists a multi-layered structure in the grain boundary phase. From outside to inside of the multi-layered structure, layers with the following phases are found in direct order: the RE-rich phase, the Fe-rich phase, and the REFe₂ phase. This multi-layered grain boundary phase structure could restrain the reduction of Hcj even in case of high ratio addition of Ce element.

In the magnet of Comparative Example 1, a REFe₂ phase and multi-layered structure was not found by the microstructure analysis for low addition ratio of Ce element (2.00wt.%). Even though the remanence (Br) was high at 1.41 T, the intrinsic coercivity (Hcj) dropped down to only 1086.54 kA/m. From the comparison of Comparative Example 1 with Implementing Example 2 including 3.00wt.% Ce (intrinsic coercivity Hcj of 1313.40 kA/m and remanence Br at 1.39 T) it can thus be deduced that a content of at least 3.00wt.% of Ce is necessary for forming the multi-layered structure and thereby enhancing the intrinsic coercivity Hcj.

In the magnet of Comparative Example 2, a large amount of REFe₂ phase was found for high addition ratio of Ce element (18wt.%). The REFe₂ phase was widely distributed between the main grains, and the multi-layered grain boundary structure was hard to form. As a consequence, the intrinsic coercivity Hcj dropped down to only 644.76 kA/m at even low remanence Br of 1.27 T.

The Ce content thus has an influence on forming the desired multi-layered grain boundary structure. In absence of the multi-layered grain boundary structure, the magnets of the Comparative Examples have lower intrinsic coercivity.

### List of Reference Signs

- 1: grains formed of main phase
- 2: RE-rich layer of grain boundary phase multi-layered structure
- 2a: width center of RE-rich layer
- 3: Fe-rich layer of grain boundary phase multi-layered structure
- 3a: width center of Fe-rich layer
- 4: REFe₂ layer of grain boundary phase multi-layered structure
- 5: thickness test location of multi-layered structure

## Claims

1. A Ce-containing and sintered NdFeB magnet comprising grains (1) composed of a RE₂Fe₁₄B-type main phase and a multi-layered grain boundary structure between the grains (1),
wherein the multi-layered grain boundary structure includes from outside to inside of the multi-layered structure and in direct order layers (2, 3, 4) composed of the following phases: a RE-rich phase, a Fe-rich phase, and a REFe₂ phase,
wherein the magnet alloy composition is a RE-T-B-M magnet alloy composition where
• RE is a rare earth metal including Ce and at least one of Nd and Pr;
• T is one or both of Fe and Co;
• B stands for boron;
• M is one or more element selected from the group consisting of Al, Cu, Ga, and Ti;
wherein the weight contents of the RE-T-B-M magnet alloy composition are set as follows:
• RE: 28.50wt.% to 35.00wt.%;
• Ce: 3.00wt.% to 15.00wt.%;
• Nd and Pr: 14.00wt.% to 29.00wt.%;
• B: 0.70wt.% to 1.20wt.%;
• Co: 0.10 wt. % to 3.00wt.%;
• M: 0.10wt. % to 3.00wt.%; and
• the residual is Fe and unavoidable impurities;
**characterised in that**
(i) in the RE-rich phase, RE takes an atomic proportion of 50.0at.% to 63.0at.%, Fe plus Co takes an atomic proportion of 30.0at.% to 40.0at.%, and M takes an atomic proportion of 2.0at.% to 12.0at.%, wherein the components plus unavoidable impurities add up to 100at.%;
(ii) in the Fe-rich phase, RE takes an atomic proportion of 10.0at.% to 30.0at.%, Fe plus Co takes an atomic proportion of 65.0at.% to 85.0at.%, and M takes an atomic proportion of 1.0at.% to 7.0at.%, wherein the components plus unavoidable impurities add up to 1 00at.%;
(iii) in the REFe₂ phase, RE takes an atomic proportion of 25.0at.% to 35.0at.%, Fe plus Co takes an atomic proportion of 60.0at.% to 72.0at.%, and M takes an atomic proportion of 0.5at.% to 6.0at.%, wherein the components plus unavoidable impurities add up to 100at.%; and
wherein the RE-rich phase layer (2) has a thickness of 1nm to 21nm, the Fe-rich phase layer (3) has a thickness of 1nm to 15nm, and the REFe₂ phase layer (4) has a thickness of 8nm to 550nm.

2. The Ce-containing and sintered NdFeB magnet of claim 1,
wherein the weight contents of the RE-T-B-M magnet alloy composition are set as follows:
• RE: 29.50wt.% to 34.00wt.%, in particular 30.10wt.% to 33.50wt.%;
• Ce: 5.00wt.% to 10.00wt.%;
• Nd and Pr: 15.00wt.% to 28.00wt.%, in particular 15.30wt.% to 27.10wt.%;
• B: 0.80wt.% to 1.10wt.%, in particular 0.85 wt.% to 1.05wt.%;
• Co: 0.50 wt. % to 2.00wt. %;
• M: 0.30wt.% to 1.50wt.%, in particular 0.55wt.% to 1.20wt.%; and
• the residual is Fe and unavoidable impurities.

3. The Ce-containing and sintered NdFeB magnet of claim 2, wherein the weight contents of Al, Cu, Ga, and Ti as metallic alloy components of the RE-T-B-M magnet alloy composition are independently from each other set as follows:
Al: 0.01 wt.% to 1.00wt.%, preferably 0.05 wt.% to 0.60wt.%;
Cu: 0.01 wt.% to 1.00wt.%, preferably 0.10 wt.% to 0.50wt.%;
Ga: 0.01 wt.% to 1.00wt.%, preferably 0.10 wt.% to 0.50wt.%; and
Ti: 0.01 wt.% to 1.00wt.%, preferably 0.10 wt.% to 0.40wt.%.

4. The Ce-containing and sintered NdFeB magnet of any one of the preceding claims, wherein
(ii) in the Fe-rich phase, RE takes an atomic proportion of 12.4at.% to 26.0at.%, Fe plus Co takes an atomic proportion of 68.1at.% to 81.4at.%, and M takes an atomic proportion of 1.3at.% to 6.2at.% , wherein the components plus unavoidable impurities add up to 100at.%; and/or
(iii) in the REFe₂ phase, RE takes an atomic proportion of 28.1at.% to 33.8at.%, Fe plus Co takes an atomic proportion of 61.4at.% to 69.8at.%, and M takes an atomic proportion of 0.6at.% to 4.8at.% , wherein the components plus unavoidable impurities add up to 100at.%.

5. A manufacturing method of a Ce-containing and sintered NdFeB magnet comprising grains composed of a RE₂Fe₁₄B-type main phase and a multi-layered grain boundary structure between the grains as defined in any one of the preceding claims, the method including the following steps:
a) Preparing alloy flakes of the magnet alloy composition by a strip casting process, subjecting the alloys flakes to hydrogen decrepitation und pulverizing the product by jet milling to obtain an alloy powder, wherein the magnet alloy composition is a RE-T-B-M magnet alloy composition where
• RE is a rare earth metal including Ce and at least one of Nd and Pr;
• T is one or both of Fe and Co;
• B stands for boron;
• M is one or more element selected from the group consisting of Al, Cu, Ga, and Ti;
And wherein the weight contents of the RE-T-B-M magnet alloy composition are set as follows:
• RE: 28.50wt.% to 35.00wt.%;
• Ce: 3.00wt.% to 15.00wt.%;
• Nd and Pr: 14.00wt.% to 29.00wt.%;
• B: 0.70wt.% to 1.20wt.%;
• Co: 0.10 wt. % to 3.00wt.%;
• M: 0.10wt. % to 3.00wt.%; and
• the residual is Fe and unavoidable impurities;
b) Pressing the magnetic powder into a green compact under a magnetic field for orientation followed by cold isostatic pressing;
c) sintering the green compact at 950°C to 1100°C for 2 to 15h, preferably at 1000°C to 1050°C for 4 to 12h, for example, 1010°C for a duration time of 6 hours;
d) After sintering, subjecting the obtained sintered NdFeB magnets to an annealing treatment,
**characterised in that**
the annealing treatment consists of three steps, wherein
- in a first step of the annealing treatment a temperature is in the range of 600°C to 750°C, preferably 630°C to 730°C, for example 650°C, for 1h to 5h, preferably 2h to 4h, for example 3h,
- in a second step of the annealing treatment a temperature is in the range of 800°C to 950°C, preferably 820°C to 930°C, for example 850°C, for 1h to 5h, preferably 2h to 4h, for example 3h, and
- in a third step of the annealing treatment a temperature is in the range of 420°C to 560°C, preferably 450°C to 540°C, for example 480°C, for 1h to 5h, preferably 2h to 4h, for example 3h.

## Patentansprüche

1. Ce-haltiger und gesinterter NdFeB-Magnet, umfassend Körner (1), die aus einer Hauptphase vom Typ RE₂Fe₁₄B und einer mehrschichtigen Korngrenzstruktur zwischen den Körnern (1) bestehen,
wobei die mehrschichtige Korngrenzstruktur von außen nach innen bezüglich der mehrschichtigen Struktur und in direkter Reihenfolge Schichten (2, 3, 4) umfasst, die aus den folgenden Phasen bestehen: einer RE-reichen Phase, einer Fe-reichen Phase und einer REFe₂-Phase,
wobei die Magnetlegierungszusammensetzung eine RE-T-B-M-Magnetlegierungszusammensetzung ist, in der
• RE ein Seltenerdmetall ist, das Ce und mindestens eines von Nd und Pr umfasst;
• T eines oder beide von Fe und Co ist;
• B für Bor steht;
• M eines oder mehrere Elemente ist, die aus der Gruppe bestehend aus Al, Cu, Ga und Ti ausgewählt sind;
wobei die Gewichtsanteile der RE-T-B-M-Magnetlegierungszusammensetzung wie folgt festgelegt sind:
• RE: 28,50 Gew.-% bis 35,00 Gew.-%;
• Ce: 3,00 Gew.-% bis 15,00 Gew.-%;
• Nd und Pr: 14,00 Gew.-% bis 29,00 Gew.-%;
• B: 0,70 Gew.-% bis 1,20 Gew.-%;
• Co: 0,10 Gew.-% bis 3,00 Gew.-%;
• M: 0,10 Gew.-% bis 3,00 Gew.-%; und
• der Rest Fe und unvermeidbare Verunreinigungen ist;
**dadurch gekennzeichnet, dass**
(i) in der RE-reichen Phase RE einen Atomanteil von 50,0 at.% bis 63,0 at.% einnimmt, Fe plus Co einen Atomanteil von 30,0 at.% bis 40,0 at.% einnehmen und M einen Atomanteil von 2,0 at.% bis 12,0 at.% einnimmt, wobei die Komponenten plus unvermeidbare Verunreinigungen insgesamt 100 at.% ergeben;
(ii) in der Fe-reichen Phase RE einen Atomanteil von 10,0 at.% bis 30,0 at.% einnimmt, Fe plus Co einen Atomanteil von 65,0 at.% bis 85,0 at.% einnehmen und M einen Atomanteil von 1,0 at.% bis 7,0 at.% einnimmt, wobei die Komponenten plus unvermeidbare Verunreinigungen insgesamt 100 at.% ergeben;
(iii) in der REFe₂-Phase RE einen Atomanteil von 25,0 at.% bis 35,0 at.% einnimmt, Fe plus Co einen Atomanteil von 60,0 at.% bis 72,0 at.% einnehmen und M einen Atomanteil von 0,5 at.% bis 6,0 at.% einnimmt, wobei die Komponenten plus unvermeidbare Verunreinigungen insgesamt 100 at.% ergeben; und
wobei die RE-reiche Phasenschicht (2) eine Dicke von 1 nm bis 21 nm, die Fe-reiche Phasenschicht (3) eine Dicke von 1 nm bis 15 nm und die REFe₂-Phasenschicht (4) eine Dicke von 8 nm bis 550 nm aufweist.

2. Ce-haltiger und gesinterter NdFeB-Magnet nach Anspruch 1,
wobei die Gewichtsanteile der RE-T-B-M-Magnetlegierungszusammensetzung wie folgt festgelegt sind:
• RE: 29,50 Gew.-% bis 34,00 Gew.-%, insbesondere 30,10 Gew.-% bis 33,50 Gew.-%;
• Ce: 5,00 Gew.-% bis 10,00 Gew.-%;
• Nd und Pr: 15,00 Gew.-% bis 28,00 Gew.-%, insbesondere 15,30 Gew.-% bis 27,10 Gew.-%;
• B: 0,80 Gew.-% bis 1,10 Gew.-%, insbesondere 0,85 Gew.-% bis 1,05 Gew.-%;
• Co: 0,50 Gew.-% bis 2,00 Gew.-%;
• M: 0,30 Gew.-% bis 1,50 Gew.-%, insbesondere 0,55 Gew.-% bis 1,20 Gew.-%; und
• der Rest Fe und unvermeidbare Verunreinigungen ist.

3. Ce-haltiger und gesinterter NdFeB-Magnet nach Anspruch 2, wobei die Gewichtsanteile von Al, Cu, Ga und Ti als metallische Legierungskomponenten der RE-T-B-M-Magnetlegierungszusammensetzung unabhängig voneinander wie folgt festgelegt sind:
Al: 0,01 Gew.-% bis 1,00 Gew.-%, vorzugsweise 0,05 Gew.-% bis 0,60 Gew.-%;
Cu: 0,01 Gew.-% bis 1,00 Gew.-%, vorzugsweise 0,10 Gew.-% bis 0,50 Gew.-%;
Ga: 0,01 Gew.-% bis 1,00 Gew.-%, vorzugsweise 0,10 Gew.-% bis 0,50 Gew.-%; und
Ti: 0,01 Gew.-% bis 1,00 Gew.-%, vorzugsweise 0,10 Gew.-% bis 0,40 Gew.-%.

4. Ce-haltiger und gesinterter NdFeB-Magnet nach einem der vorstehenden Ansprüche, wobei
(ii) in der Fe-reichen Phase RE einen Atomanteil von 12,4 at.% bis 26,0 at.% einnimmt, Fe plus Co einen Atomanteil von 68,1 at.% bis 81,4 at.% einnehmen und M einen Atomanteil von 1,3 at.% bis 6,2 at.% einnimmt, wobei die Komponenten plus unvermeidbare Verunreinigungen insgesamt 100 at.% ergeben; und/oder
(iii) in der REFe₂-Phase RE einen Atomanteil von 28,1 at.% bis 33,8 at.% einnimmt, Fe plus Co einen Atomanteil von 61,4 at.% bis 69,8 at.% einnehmen und M einen Atomanteil von 0,6 at.% bis 4,8 at.% einnimmt, wobei die Komponenten plus unvermeidbare Verunreinigungen insgesamt 100 at.% ergeben.

5. Verfahren zur Herstellung eines Ce-haltigen und gesinterten NdFeB-Magneten, der Körner umfasst, die aus einer Hauptphase vom Typ RE₂Fe₁₄B und einer mehrschichtigen Korngrenzenstruktur zwischen den Körnern bestehen, wie in einem der vorstehenden Ansprüche definiert, wobei das Verfahren die folgenden Schritte umfasst:
a) Herstellen von Legierungsflocken der Magnetlegierungszusammensetzung durch ein Bandgießverfahren, Unterziehen der Legierungsflocken einer Wasserstoffdekrepitation und Pulverisieren des Produkts durch Strahlmahlen, um ein Legierungspulver zu erhalten, wobei die Magnetlegierungszusammensetzung eine RE-T-B-M-Magnetlegierungszusammensetzung ist, in der
• RE ein Seltenerdmetall ist, das Ce und mindestens eines von Nd und Pr enthält;
• T eines oder beide von Fe und Co ist;
• B für Bor steht;
• M ein oder mehrere Elemente ist, die aus der Gruppe bestehend aus Al, Cu, Ga und Ti ausgewählt sind;
und wobei die Gewichtsanteile der RE-T-B-M-Magnetlegierungszusammensetzung wie folgt festgelegt sind:
• RE: 28,50 Gew.-% bis 35,00 Gew.-%;
• Ce: 3,00 Gew.-% bis 15,00 Gew.-%;
• Nd und Pr: 14,00 Gew.-% bis 29,00 Gew.-%;
• B: 0,70 Gew.-% bis 1,20 Gew.-%;
• Co: 0,10 Gew.-% bis 3,00 Gew.-%;
• M: 0,10 Gew.-% bis 3,00 Gew.-%; und
• der Rest Fe und unvermeidbare Verunreinigungen ist;
b) Pressen des Magnetpulvers unter einem Magnetfeld zur Ausrichtung zu einem Grünling, gefolgt von kaltisostatischem Pressen;
c) Sintern des Grünlings bei 950°C bis 1100°C für 2 bis 15 Stunden, vorzugsweise bei 1000°C bis 1050°C für 4 bis 12 Stunden, beispielsweise bei 1010°C für eine Dauer von 6 Stunden,
d) Unterziehen der erhaltenen gesinterten NdFeB-Magnete einer Glühbehandlung nach dem Sintern,
**dadurch gekennzeichnet, dass**
die Glühbehandlung aus drei Schritten besteht, wobei
- in einem ersten Schritt der Glühbehandlung eine Temperatur im Bereich von 600°C bis 750°C liegt, vorzugsweise 630°C bis 730°C, beispielsweise 650°C, für 1 bis 5 Stunden, vorzugsweise 2 bis 4 Stunden, beispielsweise 3 Stunden,
- in einem zweiten Schritt der Glühbehandlung eine Temperatur im Bereich von 800°C bis 950°C liegt, vorzugsweise 820°C bis 930°C, beispielsweise 850°C, für 1 bis 5 Stunden, vorzugsweise 2 bis 4 Stunden, beispielsweise 3 Stunden, und
- in einem dritten Schritt der Glühbehandlung eine Temperatur im Bereich von 420°C bis 560°C liegt, vorzugsweise 450°C bis 540°C, beispielsweise 480°C, für 1 bis 5 Stunden, vorzugsweise 2 bis 4 Stunden, beispielsweise 3 Stunden.

## Revendications

1. Aimant fritté NdFeB et contenant du Ce comprenant des grains (1) composés d'une phase principale de type RE₂Fe₁₄B et d'une structure de joints de grains multicouche entre les grains (1),
dans lequel la structure de joints de grains multicouche comporte à partir d'un extérieur vers un intérieur de la structure multicouche et dans un ordre direct des couches (2, 3, 4) composées des phases suivantes : une phase riche en RE, une phase riche en Fe, et une phase du REFe₂,
dans lequel la composition d'alliage d'aimant est une composition d'alliage d'aimant RE-T-B-M où
• RE est un métal de terres rares comportant du Ce et au moins un élément entre Nd et Pr;
• T est un ou deux éléments entre Fe et Co ;
• B désigne le bore ;
• M est un ou plusieurs éléments sélectionnés du groupe consistant en Al, Cu, Ga, et Ti ;
dans lequel le contenu en poids de la composition d'alliage d'aimant RE-T-B-M est défini comme suit :
• RE : 28,50 wt.% à 35,00 wt.% ;
• Ce : 3,00 wt.% à 15,00 wt.% ;
• Nd et Pr : 14,00 wt.% à 29,00 wt.% ;
• B : 0,70 wt.% à 1,20 wt.% ;
• Co : 0,10 wt.% à 3,00 wt.% ;
• M : 0,10 wt.% à 3,00 wt.% ; et
• le résidu est du Fe et des impuretés inévitables ;
**caractérisé en ce que**
(i) dans la phase riche en RE, RE prend une proportion atomique de 50,0 at.% à 63,0 at.%, Fe +Co prend une proportion atomique de 30,0 at.% à 40,0 at.%, et M prend une proportion atomique de 2,0 at.% à 12,0 at.%, dans lequel l'ensemble des composants y compris des impuretés inévitables atteint à 100 at.% ;
(ii) dans la phase riche en Fe, RE prend une proportion atomique de 10,0 at.% à 30,0 at.%, Fe +Co prend une proportion atomique de 65,0 at.% à 85,0 at.%, et M prend une proportion atomique de 1,0 at.% à 7,0 at.%, dans lequel l'ensemble des composants y compris des impuretés inévitables atteint à 100 at.% ;
(iii) dans la phase du REFe₂, RE prend une proportion atomique de 25,0 at.% à 35,0 at.%, Fe +Co prend une proportion atomique de 60,0 at.% à 72,0 at.%, et M prend une proportion atomique de 0,5 at.% à 6,0 at.%, dans lequel l'ensemble des composants y compris des impuretés inévitables atteint à 100 at.% ; et
dans lequel la couche de phase riche en RE (2) a une épaisseur de 1 nm à 21 nm, la couche de phase riche en Fe (3) a une épaisseur de 1 nm à 15 nm, et la couche de phase du REFe₂ (4) a une épaisseur de 8 nm à 550 nm.

2. Aimant fritté NdFeB et contenant du Ce selon la revendication 1,
dans lequel le contenu en poids de la composition d'alliage d'aimant RE-T-B-M est défini comme suit :
• RE : 29,50 wt.% à 34,00 wt.%, en particulier 30,10 wt.% à 33,50 wt.% ;
• Ce : 5,00 wt.% à 10,00 wt.% ;
• Nd et Pr : 15,00 wt.% à 28,00 wt.%, en particulier 15,30 wt.% à 27,10 wt.% ;
• B : 0,80 wt.% à 1,10 wt.%, en particulier 0,85 wt.% à 1,05 wt.% ;
• Co : 0,50 wt.% à 2,00 wt.% ;
• M : 0,30 wt.% à 1,50 wt.%, en particulier 0,55 wt.% à 1,20 wt.% ; et
• le résidu est du Fe et des impuretés inévitables.

3. Aimant fritté NdFeB et contenant du Ce selon la revendication 2, dans lequel le contenu en poids d' Al, Cu, Ga, et Ti comme des composants d'alliage métallique de la composition d'alliage d'aimant RE-T-B-M sont définis indépendamment les uns des autres comme suit :
Al : 0,01 wt.% à 1,00 wt.%, parfaitement 0,05 wt.% à 0,60 wt.% ;
Cu : 0,01 wt.% à 1,00 wt.%, parfaitement 0,10 wt.% à 0,50 wt.% ;
Ga : 0,01 wt.% à 1,00 wt.%, parfaitement 0,10 wt.% à 0,50 wt.% ; et
Ti : 0,01 wt.% à 1,00 wt.%, parfaitement 0,10 wt.% à 0,40 wt.%.

4. Aimant fritté NdFeB et contenant du Ce selon l'une quelconque des revendications précédentes, dans lequel
(ii) dans la phase riche en Fe, RE prend une proportion atomique de 12,4 at.% à 26,0 at.%, Fe +Co prend une proportion atomique de 68,1 at.% à 81,4 at.%, et M prend une proportion atomique de 1,3 at.% à 6,2 at.% , dans lequel l'ensemble des composants y compris des impuretés inévitables atteint à 100 at.% ; et/ou
(iii) dans la phase du REFe₂, RE prend une proportion atomique de 28,1 at.% à 33,8 at.%, Fe +Co prend une proportion atomique de 61,4 at.% à 69,8 at.%, et M prend une proportion atomique de 0,6 at.% à 4,8 at.% , dans lequel l'ensemble des composants y compris des impuretés inévitables atteint à 100 at.%.

5. Procédé de fabrication d'un aimant fritté NdFeB et contenant du Ce comprenant des grains composés d'une phase principale de type RE₂Fe₁₄B et d'une structure de joints de grains multicouche entre les grains telle que définie dans l'une quelconque des revendications précédentes, le procédé comportant les étapes suivantes :
a) Préparer des flocons d'alliage de la composition d'alliage d'aimant par un processus coulée en bande, soumettre les flocons d'alliage à une décrépitation par l'hydrogène et pulvériser le produit par un broyage à jet pour obtenir une poudre d'alliage, dans lequel la composition d'alliage d'aimant est une composition d'alliage d'aimant RE-T-B-M où
• RE est un métal de terres rares comportant du Ce et au moins un élément entre Nd et Pr;
• T est un ou deux éléments entre Fe et Co ;
• B désigne le bore ;
• M est un ou plusieurs éléments sélectionnés du groupe consistant en Al, Cu, Ga, et Ti ;
Et dans lequel le contenu en poids de la composition d'alliage d'aimant RE-T-B-M est défini comme suit :
• RE : 28,50 wt.% à 35,00 wt.% ;
• Ce : 3,00 wt.% à 15,00 wt.% ;
• Nd et Pr : 14,00 wt.% à 29,00 wt.% ;
• B : 0,70 wt.% à 1,20 wt.% ;
• Co : 0,10 wt.% à 3,00 wt.% ;
• M : 0,10 wt.% à 3,00 wt.% ; et
• le résidu est du Fe et des impuretés inévitables ;
b) Presser la poudre d'aimant pour former un compact vert sous un champs magnétique pour orientation suivie par un pressage isostatique à froid ;
c) fritter le compact vert de 950 °C à 1100 °C pendant 2 h à 15 h, parfaitement de 1000 °C à 1050 °C pendant 4 h à 12 h, par exemple, 1010 °C pendant un temps de durée de 6 heures;
d) Après le frittage, soumettre les aimants frittés NdFeB obtenus à un traitement de recuit,
**caractérisé en ce que**
le traitement de recuit consiste en trois étapes, dans lequel
- dans une première étape du traitement de recuit une température est dans une plage de 600 °C à 750 °C, parfaitement 630 °C à 730 °C, par exemple 650 °C, pendant 1 h à 5 h, parfaitement 2 h à 4 h, par exemple 3 h,
- dans une deuxième étape du traitement de recuit une température est dans une plage de 800°C à 950°C, parfaitement 820 °C à 930 °C, par exemple 850 °C, pendant 1 h à 5 h, parfaitement 2 h à 4 h, par exemple 3 h, et
- dans une troisième étape du traitement de recuit une température est dans une plage de 420 °C à 560 °C, parfaitement 450 °C à 540 °C, par exemple 480 °C, pendant 1 h à 5 h, parfaitement 2 h à 4 h, par exemple 3 h.
